

## UNITED STATES PATENT OFFICE

2,159,510

METHOD OF COATING COPPER OR ITS  
ALLOYS WITH TIN

Arnold E. Pavlish and John D. Sullivan, Columbus, Ohio, assignors to Battelle Memorial Institute, Columbus, Ohio, a corporation of Ohio

No Drawing. Application April 5, 1937.  
Serial No. 135,081

## 5 Claims. (Cl. 91—68.3)

Our invention relates to a method of coating copper or its alloys with tin. More specifically, it relates to a method of coating by an immersion process, without the use of an electric current from an outside source or of a contact metal within the bath to be utilized.

Copper and its alloys have an enviable position in the architectural and industrial fields because of their intrinsic physical and chemical properties. For many purposes, however, a coating of another metal over the copper or alloy is desired to increase resistance to corrosion or for enhancing the beauty or utility of the article. Tin has found wide application for this purpose.

15 Copper and its alloys find wide use in the plumbing industry. Water frequently attacks tubes or pipes, giving rise to what is commonly termed "green water". The rate of formation of metallic salts that cause green water varies with the pipes used, the purity of the water, the gases dissolved therein, temperature, and other factors. If water is continuously flowing through pipes, the concentration of salts either in solution, in colloidal form, or in mechanical suspension is usually not great enough to cause noticeable coloring of the water or staining of plumbing fixtures. If the flow is intermittent, as it usually is in domestic buildings, the concentration may become high enough to give an ugly 20 color to the water or to stain the fixtures. Formation of color stains is frequently accentuated by toilet or laundry soaps which form insoluble colored copper soaps.

35 In the prior art, attempts have been made to coat the inside of pipes and tubes with metallic tin by a hot sweating process which involves the application of molten tin to the inner walls of said pipes or tubes by a mechanical swabbing operation. This method is expensive and results in a coating which is neither uniform in thickness nor in surface contour. Moreover, such a method is limited to relatively short sections of such pipe or tubing. Likewise, it is not practicable for coating the inside of a coil of pipe.

40 For enhancing the beauty of various copper or copper alloy articles in the prior art, recourse has been had to the electrodeposition of tin. While this method is satisfactory for many purposes, it is subject to certain important limitations. For example, it is not practicable for use in the coating of the inner walls of tubes or pipes of appreciable length, or distorted shape. Also, it is difficult to electroplate satisfactorily large articles, especially when they are of complicated 45 shape and design. Likewise, all coatings of tin

which are produced by electrodeposition tend to be defective because they do not cover completely the surface to which they are applied and commonly have pinhole openings at numerous points in the coating.

5 In the past, certain small articles, such as pins, safety pins, thimbles, buttons and the like have been coated with tin by what is known as contact-immersion processes. These processes consist of placing the articles in contact with a metal such as zinc, while immersed in a solution such as a tin salt. This contact metal sets up a galvanic cell, so that in effect the process is one of electrodeposition wherein the electric current is generated by chemical means within the bath. 10 These processes have very limited application and are not suitable for coating the interiors of pipes or tubes.

15 In the art of deposition by the contact process, as commonly practiced, the baths utilized normally contain such combinations as a saturated solution of cream of tartar containing stannous chloride, a solution containing from 20 to 30 grams of ammonium alum and 1 to 2 grams of stannous chloride per liter, or a sodium stannite 20 solution containing about 7 grams per liter of sodium cyanide. Coatings obtained from such baths are ordinarily extremely thin, do not have good covering powers and are comparatively expensive. Furthermore, these coatings can be applied only to small and relatively simple articles 25 and cannot be applied to pipes and tubes of appreciable length and particularly to the interior thereof. Likewise, these baths must be operated usually at elevated temperatures, approaching 30 the boiling point and the tin salts are unstable under these conditions of operation, with the result that the baths rapidly become depleted. Likewise, the time required for coating with these 35 baths is usually long, frequently amounting to 40 several hours.

45 One of the objects of this invention is to obtain coatings of tin on copper or its alloys or copper alloy coated articles by a simple and relatively inexpensive process wherein the coating may be produced in a relatively brief time.

Another object of this invention is to produce such a coating of tin on the materials specified by the use of a bath at atmospheric temperature and without the use of an electric current.

50 Another object of this invention is to produce coatings of tin on materials of the type indicated which will be sufficiently thick and which will have ample covering power.

5

20

25

30

35

40

45

50

55

Other objects will appear from the following description and claims.

Our invention involves the discovery that tin coating can be applied to copper or its alloys by an immersion process at ordinary temperatures and without the use of electric current from the outside or any contact metal within the baths. The invention is based on the fact that baths containing certain ingredients in selected proportions will be effective to produce a coating of tin upon a copper or copper alloy without the use of any contact metal or of any electric current from the outside.

It has been discovered that, if a bath contains stannous tin and a sufficiently high concentration of cyanide, coatings of excellent quality can be produced on copper or copper alloys with the bath at room temperature. Although the essential characteristics of the bath require the presence of a high concentration of cyanide and the presence of stannous tin, the latter can be present in the solution in various forms. Likewise, different raw materials can be utilized to prepare the bath. Thus, it is possible to utilize a bath comprising sodium stannite and sodium cyanide or a bath of stannous tartrate or citrate and sodium cyanide. However, these baths are illustrative only and, although they do not exhaust the possible sources of stannous tin, they show the wide range of materials that can be used.

It is obvious, of course, that sodium stannite may be prepared by adding to the bath required amounts of stannous salts such as stannous chloride and sodium hydroxide. Likewise, tin tartrate can be made from tartaric acid and a suitable tin salt. Potassium, ammonium or other alkali salts can be used instead of sodium salts.

One form of our method will be illustrated by considering a sodium stannite-sodium cyanide bath. We have prepared baths of sodium stannite by reaction of stannous chloride and sodium hydroxide according to the following reaction:



A sodium stannite bath so prepared is ready for use on addition of sodium cyanide. The concentration of sodium stannite can vary from  $\frac{1}{2}$  gram per liter to a solution substantially saturated. In fact, the concentration of sodium stannite may be lower than  $\frac{1}{2}$  gram per liter but, if so, the solution becomes depleted quite rapidly on use. The concentration of cyanide must be high, but the lower limit that can be used varies with the time allotted for coating. The following example will illustrate the concentration of sodium cyanide that can be used under varying conditions: A bath was prepared containing 5 grams per liter  $\text{SnCl}_2 \cdot 2\text{H}_2\text{O}$  and 5.6 grams per liter  $\text{NaOH}$ . The cyanide concentration was varied. A solution containing 5 grams per liter  $\text{NaCN}$  at room temperature gave but little visible coating in less than one hour, and the coating secured in that time was thin and incomplete. The surface of the copper was not protected. When the concentration of  $\text{NaCN}$  was 15 grams per liter, a visible coating was obtained in about four to five minutes, but immersion for approximately an hour was required to give complete and adequate coverage. At 25 grams  $\text{NaCN}$  per liter, a visible coating was obtained in two minutes, and satisfactory coverage was obtained in ten minutes or less. At 50 grams and above per liter, visible coatings were obtained in one minute or less. We have made coatings with solutions containing as much as 200 grams  $\text{NaCN}$  per liter. The

example above is illustrative only and our invention is not limited to the concentration of  $\text{SnCl}_2$  or  $\text{NaOH}$  given in the example.

In the operation of our process, the copper or copper alloy article is preferably properly cleaned or cleaned and pickled in the manner followed for preparing such articles for plating, coating or the like, although in some instances such cleaning or cleaning and pickling operations are not absolutely necessary. In fact, the solution itself has cleansing properties. The article is immersed in the stannite-cyanide bath. Immediately upon immersion, tin commences to deposit on the article in plate-like form. In many cases, a satisfactory coating is obtained in one minute or less, although in some cases a longer period is required. In general, the longer the period of immersion, the heavier will be the coat obtained. Although we do not care to be bound by any particular theory, we believe that the coating results from an electrochemical replacement, with the copper going into solution and the tin plating out. The bath may be operated at room temperature.

If it is desired to coat the inside of pipes, tubes or coils of pipes, this may be effected by the simple process of passing the bath solution through them. Thus, it is possible to coat the inside of such pipes, tubes or coils of pipe without coating the outside.

Other cyanide baths are used in much the same manner as the stannite-cyanide bath. An important characteristic is high cyanide content of the bath. Tin tartrate immersion plating baths may be made by using varying amounts of sodium stannite, tartaric acid, and sodium cyanide. Stannous chloride may be substituted for sodium stannite. In the preparation of a bath from stannous chloride, tartaric acid, and sodium cyanide, the concentration of stannous chloride can be varied over wide limits but, in order to get satisfactory performance, the concentration of tartaric acid and cyanide must be controlled more carefully. For example, with a bath containing 5 grams per liter  $\text{SnCl}_2 \cdot 2\text{H}_2\text{O}$  and 20 grams per liter tartaric acid, the addition of  $\text{NaCN}$  causes a precipitation of part of the tin from solution. However, such a bath will yield coatings, provided the concentration of  $\text{NaCN}$  exceeds 35 grams per liter. However, increasing the concentration to 50 grams or more  $\text{NaCN}$  per liter effected much more rapid coating. Addition of sufficient tartaric acid permits making a solution from which the tin is not precipitated on addition of  $\text{NaCN}$ , and which yields satisfactory coatings. This will be illustrated by the following examples: A bath was made containing 5 grams per liter  $\text{SnCl}_2 \cdot 2\text{H}_2\text{O}$ , 50 grams per liter  $\text{NaCN}$  and varying amounts of tartaric acid. With no tartaric acid, the solution was alkaline, and a heavy sludge formed. With 10 grams per liter, the solution was still alkaline and a heavy sludge also formed. With 30 grams per liter, the sludge was less but the solution was still alkaline. With 50 and 75 grams per liter, the sludges were very slight and the solutions were alkaline. When 100 grams per liter was used, the sludge was slight but the solution was acidic. The solutions deposited tin on copper by immersion so long as the solutions were alkaline in nature. The prerequisites of a tartaric-cyanide bath, therefore, are sufficient tartaric acid or soluble tartrate to prevent precipitation of tin on addition of  $\text{NaCN}$ , and sufficient  $\text{NaCN}$  to maintain the solution alkaline in nature. An excess of cyanide over that required to make

the solution alkaline is desirable to effect rapid coating. The examples above are illustrative only, and those skilled in the art can choose different amounts and concentrations on the basis of the disclosure.

5 Citric acids or soluble citrates can be used in place of tartaric acid. The results are similar in nature if equivalent amounts are used.

Tin coatings can be put on copper coated articles as well as on copper itself. Thus, it is possible to coat iron or steel with copper or its alloys by well-known means and to thereafter apply a tin coating to the thus-prepared surface by the method of this invention.

10 It has also been discovered in some cases that superior coatings can be obtained by applying a coating in the manner described above and then heating the tin-coated material for a period at a low temperature, and then applying a second coating by again immersing the article in the coating solution. The procedure may be repeated 15 several times, if desirable. We have found that by heating at about 230° C. for a time sufficient to bring the article to temperature or longer gives the desired results. In some cases, it is desirable to heat substantially above 230° C. to effect 20 alloying of the tin with the base metal.

15 As pointed out, our invention in its preferred form contemplates applying a coating of tin to 25 copper or its alloys by immersion in a solution containing stannous tin and appreciable amounts of cyanide. As also pointed out, the bath may be operated at room temperatures but the invention is not limited thereto. We may, however, 30 for example, carry on the coating operation at temperatures up to the boiling point of the solution used.

35 This invention is particularly advantageous because it yields coatings that are continuous and with a highly metallic sheen. In fact, coatings are equal to and, in many cases, superior 40 in appearance to those obtained by electroplating. The bath can be operated at low temperatures and does not require the expensive method of 45 heating necessary in prior art contact-immersion baths. It is more stable than prior art contact-immersion baths. Furthermore, the necessity of using a contact metal is eliminated, thus simplifying the operation of the bath and decreasing 50 the cost of operation. The quality of coating, especially as regards continuity and freedom from pinholes, exceeds that of coatings from prior art contact-immersion baths. Coatings are obtained

5 by a simple operation. This is decidedly advantageous since by this method the inside of coils of pipe can be coated, whereas such an operation cannot be effectively performed by any prior art operation, including swabbing with molten tin, electroplating, or immersion by the contact process. It is also possible by the process of this invention to coat the inside of pipe, only, thus effecting a material saving in the amount of tin used.

10 It has been found that trouble due to green water in plumbing fixtures may be eliminated by application of a coating of tin to the inside of pipes or tubes by the method of this invention. It has also been possible by use of this invention 15 to coat various copper and brass articles to give a bright metallic tin coating that is markedly resistant to atmospheric corrosion. In short, this invention has resulted in the production of a protective or decorative coating on articles of 20 copper or its alloys or on copper or copper alloy coated articles at a remarkably low cost and in a simple manner.

25 It is within the scope of our invention to use, instead of sodium cyanide or hydroxide, other soluble cyanides or hydroxides, such as sodium, potassium, ammonium. Likewise, instead of stannous chloride, other stannous salts may be used, for example, the sulphate.

30 Having thus described our invention, what we claim is:

1. The method of forming an adherent immersion coating of tin on the surface of copper or its alloys, said method consisting essentially in contacting said surface with an alkaline aqueous 35 solution containing dissolved tin in the stannous condition and a soluble cyanide, the cyanide being in a concentration greater than 7 grams per liter.

2. The method of claim 1, wherein the said 40 solution also contains a substance selected from the group consisting of tartaric acid, tartrates, citric acid, and citrates.

3. The method of claim 1, wherein the tin-coated surface produced is heated to a temperature of at least 230° C. and the coating process 45 is repeated.

4. The method of claim 1, wherein the tin is present in the solution as sodium stannite.

5. The method of claim 1, wherein the said 50 cyanide is sodium cyanide.

ARNOLD E. PAVLISH.  
JOHN D. SULLIVAN.